

# United States Patent [19]

Holtzberg et al.

[11] 4,433,652

[45] Feb. 28, 1984

[54] COMPOSITE VALVE AND PROCESS

[75] Inventors: Matthew W. Holtzberg, Ringwood, N.J.; Lawrence D. Spaulding, Naperville, Ill.

[73] Assignee: Standard Oil Company, Chicago, Ill.

[21] Appl. No.: 387,322

[22] Filed: Jun. 11, 1982

[51] Int. Cl.<sup>3</sup> ..... F01L 3/02

[52] U.S. Cl. ..... 123/188 AA; 29/156.7 R; 264/268

[58] Field of Search ..... 123/188 AA, 90.65; 251/64 E, DIG. 3; 29/156.7 R; 264/268

[56] References Cited

## U.S. PATENT DOCUMENTS

3,748,304 7/1973 Stephens ..... 528/210

3,871,339 3/1975 Kuhn ..... 123/188 AA  
4,016,140 4/1977 Morello ..... 264/331.19  
4,224,214 9/1980 Chen ..... 264/325

## OTHER PUBLICATIONS

Wise; Charles, "Plastic Engine Is Off and Running", *Machine Design*, vol. 52, No. 10, (May 8, 1980), pp. 24-26.

Primary Examiner—William A. Cuchlinski, Jr.  
Attorney, Agent, or Firm—Thomas W. Tolpin; William T. McClain; William H. Magidson

[57] ABSTRACT

A lightweight composite valve is provided to decrease fuel consumption, attenuate noise, and permit increased speed of operation.

44 Claims, 5 Drawing Figures







## COMPOSITE VALVE AND PROCESS

## BACKGROUND OF THE INVENTION

This invention relates to engines, and more particularly, to engine parts and a process for making the same.

Traditionally, engines have been made of metal, usually steel or cast iron. Steel and cast iron engines are useful, except they are quite heavy and consume considerable amounts of gasoline or diesel fuel. Conventional engines exert large compressive forces, considerable torque, and substantial secondary harmonic vibrations which have to be damped by counterbalancing pistons, flywheels, dampeners, etc. The moving metal parts of cast iron and steel engines generate high centrifugal, reciprocating, and inertial forces, momentum, and loads. Generally, the weight of the engine adversely affects its performance, efficiency, and power.

Recently, it has been suggested to use plastic engine parts in automotive engines. Such suggestions have appeared in the December 1980 issue of *Automotive Industries* at pages 40-43, in an article entitled, "What . . . a Plastic Engine!?" in the May 8, 1980 issue of *Machine Design*, Volume 52, No. 10, in an article entitled, "Plastic Engine Is Off And Running," and in French Application No. 2,484,042, published Dec. 11, 1981.

An experimental prototype engine with concealed plastic engine parts was displayed at the Society of Automotive Engineers' (SAE) Show in Detroit, Mich. in February 1980.

Over the years, amide-imide polymers have been developed for use in molding and producing various products, such as wire coatings, enamels, films, impregnating materials, and cooking utensils. Typifying these prior art amide-imide products, polymers and molding processes are those described in U.S. Pat. Nos. 3,546,152; 3,573,260; 3,582,248; 3,660,193; 3,748,304; 3,753,998; 4,016,140; 4,084,144; 4,136,085; 4,186,236; 4,167,620; and 4,224,214. These prior art products, polymers, and molding processes have met with varying degrees of success.

It is, therefore, desirable to provide a lightweight engine part.

## SUMMARY OF THE INVENTION

An improved lightweight composite engine part is provided for use in gasoline and diesel powered automotive engines, truck engines, aircraft engines, marine engines, single and two cylinder engines, such as lawn mower engines, portable generators, and other internal combustion engines. The lightweight composite engine part decreases gasoline and fuel consumption, attenuates noise for quieter performance, and permits increased speed of operation. The lightweight composite engine part produces higher horsepower for its weight than conventional engine parts, while maintaining its shape, dimensional stability, and structural integrity at engine operating conditions. The lightweight composite engine part decreases centrifugal, reciprocating, and inertial forces, momentum, and load on the engine.

The composite engine part has a greater stiffness-to-weight ratio than metal, is flame resistant, and is stable to heat. The composite engine part is capable of effectively functioning at engine operating temperatures and start-up conditions during hot and cold weather. The composite engine part has high mechanical strength, thermal stability, fatigue strength, and excellent tensile, compressive, and flexural strength. The composite en-

gine part is resistant to wear, corrosion, impact, rupture, and creep, and reliably operates in the presence of engine fuels, oils, and exhaust gases.

In contrast to metals, such as cast iron, steel, aluminum, titanium, and to thermosetting resins, such as epoxy resin, the composite engine part can be injection molded. Injection molding permits closer tolerances with less secondary machining operations for production efficiency and economy. Finished surfaces of injected molded composite engine parts are of better quality and have fewer knit lines, seams, and flashes than do engine parts made from cold metal forging, casting, fabrication, or other conventional techniques. If desired, some of the composite engine parts can be insert molded or compression molded.

The lightweight composite engine part is made of durable, impact-resistant, hybrid or composite material which includes special proportions of an amide-imide resinous polymer, preferably reinforced with graphite and/or glass fibers. The amide-imide resinous polymer can also be blended with polytetrafluoroethylene (PTFE) and/or titanium dioxide. Composite engine parts which are injection molded or otherwise made from amide-imide resinous polymers have better elongation, stiffness, moduli, and strength at engine operating conditions than do other plastics, such as epoxy resin, polyimides, aramids, polyphenylene sulfide, polytetrafluoroethylene, and nylon. A particularly suitable amide-imide resinous polymer is commercially available from Amoco Chemicals Corporation under the trademark and product designation TORLON.

In the invention of this application, the composite engine part takes the form of a composite or hybrid engine valve. The composite valve has a metal valve head and an elongated, thermoplastic, amide-imide resinous polymeric valve stem. The valve head opens and closes the manifold. The valve stem is driven by a rocker arm or tappet and is connected to the valve head. The valve stem has at least one keeper-receiving groove. Keeper rings or locking keys fit on the keeper groove and wedgingly connect the valve spring retainer to the valve stem.

The valve head and stem each define connection parts. One of the connection parts has an outwardly extending threaded stud and the other connection part has stud-receiving means for threadedly receiving the stud. The stud-receiving means can be in the form of an internally threaded hole, or a coil spring positioned or molded within a recess.

The head and stem can be solid or hollow. In one embodiment, the valve head has an interior cavity and the valve stem has an enlarged insert molded foot that is shaped generally complementary to, and positioned within the cavity of, the valve head.

The thermoplastic, amide-imide resinous polymeric valve stem is preferably molded, allowed to cool below its plastic deformation temperature to solidify its shape, and then post cured by solid state polymerization to increase its strength. The valve stem can be injection molded or insert molded. The post cured valve stem is then connected to the valve head.

Preferably, the molding amide-imide resinous polymer comprises a graphite or glass fibrous reinforcing material which is axially injected into the stem-shaped cavity of a mold and oriented in the axial direction for increased strength.

Composite valve train parts, such as composite valves increase the natural frequency of the valve train. Composite valve train parts are more stable at engine operating conditions, minimize floating, and substantially prevent the valve train from getting out of synchronization with the cam. Composite valve trains produce less deflection and distortion, and enhance better cam timing.

A more detailed explanation of the invention is provided in the following description and appended claims taken in conjunction with the accompanying drawings.

#### BRIEF DESCRIPTION OF THE DRAWINGS

FIG. 1 is a cross-sectional view of an automotive engine with a composite valve in accordance with principles of the present invention;

FIG. 2 is a perspective view of the composite valve;

FIG. 3 is an assembly view of the composite valve with the valve stem shown partly in cross-section;

FIG. 4 is an enlarged cross-sectional view of the composite valve taken substantially along line 4—4 of FIG. 2; and

FIG. 5 is a cross-sectional view of an insert molded composite valve in accordance with principles of the present invention.

#### DETAILED DESCRIPTION OF THE PREFERRED EMBODIMENT

The automotive engine 10 of FIG. 1 has lightweight composite engine parts to reduce its weight, decrease fuel consumption, and improve engine performance. Engine 10 is a gasoline powered, four stroke, spark ignition engine. The illustrated engine is a V-6 engine with 6 cylinders arranged in a V-shaped firing pattern.

While the composite engine parts are described hereinafter with particular reference to the illustrated engine, it will be apparent that the engine parts can also be used in other types of gasoline powered automotive engines, as well as in diesel powered automotive engines, truck engines, aircraft engines, marine engines, locomotive engines, lawn mower engines, portable generators, and other internal combustion engines. The composite engine parts can be used in 1, 2, 4, 6, 8 or more cylinder engines including V-arranged cylinder engines, aligned cylinder engines, horizontally opposed cylinder engines, rotary engines, etc.

As shown in FIG. 1, engine 10 has a cast iron block 11 and head 12. The block has many chambers including a cooling chamber 13 and six combustion chambers 14 which provide cylinders. The head has an exhaust manifold and an intake manifold 16 which communicate with the cylinders and an overhead carburetor (not shown). Extending below the block is an oil pan 18. Extending above the head is a rocker arm cover 20. A distributor 22 with an internal set of spark plugs (not shown) is provided to ignite the gaseous air mixture in the cylinders.

A metal crankshaft 24 drives the pistons 26 through connecting rods 28. A counterweight 30 on crankshaft 24 balances the pistons. The crankshaft 24 drives a metal camshaft 32 through a set of timing gears 34 and 36. The timing gears include a crankshaft gear or drive pulley 34 mounted on the crankshaft 24, and a camshaft gear or driven pulley 36 mounted on the camshaft 32. A fabric reinforced, rubber timing belt 38 or timing chain drivingly connects the crankshaft gear 34 and the camshaft gear 36. The camshaft gear 36 has twice the diameter and twice as many teeth as the crankshaft gear 34, so that the camshaft 18 moves at one-half the speed of the

crankshaft. In some types of engines, the crankshaft gear drives the camshaft gear directly without a timing belt or timing chain.

Metal cams 40 are mounted on the camshaft 32 to reciprocatingly drive the valve trains 46. There are two or four valve trains per cylinder depending on the type of engine. Each valve train has a valve lifter 48, a push rod 50, a rocker arm 52, a valve spring retainer 54, a compression spring 56, and a valve 58 which opens and closes the exhaust manifold or the intake manifold 16. The intake valve 58 opens and closes the intake manifold 16. The exhaust valve opens and closes the exhaust manifold. The lifter 48 rides upon and follows the cam 40. The push rod 50 is seated in a recess of the lifter and is connected to the rocker arm 52 by a threaded stud 60 and nut 62. The bottom end of the stud 60 is shaped complementary to the top end of the push rod to securely receive and engage the push rod. The rocker arm 52 pivots upon a rocker arm shaft, fulcrum or pin 62 and reciprocatingly drives the valve stem 64 of the valve 58.

The piston 26 reciprocatingly slides against a metal liner that provides the cylinder walls. A set of piston rings is press fit or snap fit on the head of the piston. The piston rings include a compression ring 66, a barrier ring 68, and an oil scraper ring 70. The piston is pivotally connected to the connecting rod 28 through a wrist pin 72 and a bushing 74. The connecting rod is pivotally connected to the crankshaft 24 through a split ring metal bearing 76.

30 In a four stroke internal combustion engine, such as the illustrated engine, each piston has an intake stroke, a compression stroke, a power stroke, and an exhaust stroke. During the intake stroke, the piston moves downward and the inlet valve is opened to permit a gaseous air mixture to fill the combustion chamber. During the compression stroke, the intake and exhaust valves are closed and the piston moves upward to compress the gaseous air mixture. During the power stroke, the spark plug is ignited to combust the gaseous air mixture in the combustion chamber and the rapidly expanding combustion gases drive the piston downward. During the exhaust stroke, the exhaust valve is opened and the piston moves upward to discharge the combustion gases (exhaust gases).

45 The pistons, as well as connecting rods, wrist pins, barrier piston rings, push rods, rocker arms, valve spring retainers, intake valves, and timing gears, can be made of metal, although it is preferred that they are at least partially made of a thermoplastic, amide-imide resinous polymer to reduce the weight of the engine. Such amide-imide engine parts are referred to as composite engine parts. In some engines, the exhaust valve can also be at least partially made of a thermoplastic, amide-imide resinous polymer.

55 As shown in FIGS. 2-4, the composite, hybrid intake valve 58 has a thermoplastic, amide-imide resinous polymeric elongated valve stem 64 and has a metal or ceramic cap or head 100 to withstand the pressures and temperatures exerted during ignition and combustion.

60 The valve stem is reciprocatingly driven by a rocker arm or tappet. The valve head opens and closes the intake manifold. The composite valve is approximately 70% to 75% lighter than conventional metal valves. Advantageously, the thermoplastic stem and metal head 65 maintain their structural shape and integrity at engine operating conditions. The coefficient and rate of thermal expansion and contraction of the amide-imide polymeric valve stem are similar to those of the metal head,

so that the thermoplastic valve stem expands and contracts compatibly with the metal head at engine operating conditions.

The valve head 100 has a generally planar or flat circular disc or face 102 with flared, concave, semi-hyperboloid shaped sidewalls 104 which converge towards the disc. The valve head is substantially solid and is preferably made of aluminum, steel or titanium. The sidewalls provide a pedestal with an outwardly extending upright, threaded stud 106. The stud 106 threadedly engages a coil spring 108, such as helical coil spring or a helicoil compression spring, snuggly seated in a recess or hole 110 at the end of the valve stem 64. While the illustrated shaped valve head is preferred for the engine illustrated in FIG. 1, for other engines it may be desirable to use a different shaped valve head.

The valve stem has at least one keeper-receiving groove 112 in proximity to its unattached free end to receive split keeper rings or locking keys which wedge against and connect the valve spring retainer to the valve stem. The valve stem can have more than one keeper groove to adjust the height and pressure of the valve spring retainer. In the illustrative embodiment there are four keeper grooves.

The composite, hybrid intake valve 120 shown in FIG. 5 is similar to the composite hybrid valve shown in FIGS. 2-4, except that the thermoplastic, amide-imide resinous polymeric valve stem is insert molded into a hollow aluminum, steel or titanium valve head 124. When so formed, the valve stem has an enlarged insert molded bead foot or stem head 126 which is shaped complementary to, and positioned within, the outwardly flared cavity 128 of the valve head 124. The insert molded foot 126 has a maximum thickness or diameter substantially greater than the minimum thickness of the neck or throat 130 of the valve head to prevent the valve stem from being removed from the valve head 124. The illustrated foot 128 has a frusto-conical shape with a generally planar, or flat, circular base 132. While the illustrated foot is preferred for best results, other shaped feet can be used, if desired.

The valve stem 64 shown in FIGS. 2-4 is preferably injection molded for closer tolerances, minimized secondary machining operations and enhanced strength. The polymer is preferably injected in the axial direction of the valve stem to axially orient the polymer for increased strength. The injection molding temperature (polymer melt temperature) of the polymer is preferably from 630° F. to 665° F., which is above the plastic deformation temperature of the amide-imide polymer. The molded valve stem should be allowed to cool below its plastic deformation temperature to solidify its shape and polymeric orientation. The total molding and cooling time ranges from 30 to 120 seconds, depending on the grade of polymeric resin and the desired cross-sectional thickness of the valve stem.

The valve stem 122 of FIG. 5 is insert molded into the cavity 128 of the valve head 124. Insert molding also attains close tolerances, minimizes secondary machining operations and increases the structural strength of the molded valve. The polymer should also be injected along the axis of the valve stem for increased strength. The injection molding temperature and time, as well as the cooling step and time, are similar to injection molding.

The cooled molded engine part providing the blank is then post cured by solid state polymerization by progressively heating the molded engine part below its

melting temperature to enhance its dimensional strength and integrity. The specific time and temperatures depend upon the desired size of the molded part.

In the preferred method of post curing, the molded engine part is preheated in the presence of a circulating gas in an oven for a period of time such that a major portion of the volatiles contained in the injection molded engine part are vaporized and removed, while simultaneously increasing the deflection temperature of the polymer from about 15° F. to 35° F. without deformation of the engine part. Preheating can be carried out by heating the molded part from an initial temperature to a final temperature with either continuous or stepwise increases in temperature over a period of time, or at a single temperature, for a sufficient time to vaporize and remove the volatiles and increase the polymer's deflection temperature.

Imidization, cross-linking and chain extension take place during preheating. Continuous or stepwise preheating increases tensile strength and elongation properties of the molded engine parts.

In order to enhance the physical properties of smaller molded engine parts, it is preferred to continuously preheat the molded part from an initial temperature of 300° F. to 330° F. to a final preheating temperature of 460° F. to 480° F. for about 40 to 60 hours. Alternatively, the molded engine part can be preheated in a stepwise manner from an initial preheating temperature of 300° F. to 330° F. for 20 to 30 hours to a final preheating temperature of 410° F. to 430° F. for 20 to 30 hours.

Generally, the molded part is heated (post cured) at a temperature of about 330° F. for 24 hours, about 475° F. for 24 hours, and about 500° F. for 24 hours. More specifically, the molded article is heated in the presence of a circulating gas at about 5° F. to 25° F., and preferably about 5° F. to 15° F., below the increased deflection temperature of the polymer for a period of time such that substantial imidization, chain extension and cross-linking take place without deformation of the molded article.

As a result of such heating, water and gases continue to be generated and removed, and the molecular weight and deflection temperature of the polymer are increased. Heating is continued for a period of time sufficient to increase the deflection temperature by about 15° F. to 35° F. Preferably, the heating is at a temperature ranging from about 450° F. to 490° F. for a period of at least 20 hours. Thereafter, the temperature is increased to about 5° F. to 25° F. below the polymer's new deflection temperature and held at the new temperature for a sufficient time to increase the polymer's deflection temperature by about 15° F. to 35° F. Preferably, such heating is at about 480° F. to 520° F. for a period of at least 20 hours.

Heating is continued in this manner to increase the polymer's deflection temperature to its maximum attainable value without deformation of the molded article. The final heating stage is carried out at about 5° F. to 25° F., and preferably from about 5° F. to 15° F., below the maximum attainable temperature for at least 20 hours, and most preferably at least 40 hours. The heated part is then cooled.

In order to best enhance the physical properties of the molded engine part, it is preferred to heat the molded part from about 460° F. to about 480° F. for about 20 to 30 hours, then from about 490° F. to 510° F. for about 20 to 30 hours, and subsequently from about 495° F. to about 525° F. for about 20 to 60 hours.

Post curing should be carried out in the presence of a circulating gas which flows through and around the molded engine part to remove water and gases from the polymeric resin. The amount of circulation and the circulation flow pattern should be coordinated to maximize removal of water and the gases without causing substantial variations in temperature. While inert gases, such as nitrogen, can be used, it is preferred that the circulating gas be an oxygen-containing gas, most preferably air, because oxygen tends to facilitate cross-linking of the polymer molecules. Post curing is preferably carried out in a circulating air oven, although it can be carried out in any other suitable apparatus.

Post cured engine parts are resistant to thermal shock at temperatures of at least 500° F. and exhibit significantly improved tensile strength and elongation as compared with untreated molded, amide-imide resinous engine parts. A more detailed explanation of heat treatment by post curing is described in Chen U.S. Pat. No. 4,167,620, which is hereby incorporated by reference.

After the molded engine part (valve stem) is post cured, the thermoplastic valve stem and metal head are ground and connected together. In the composite valve of FIGS. 2-4, the connecting step is preceded by threading the stud 106, drilling a recess 100 at the end of the stem 64 and placing a coil spring in the recess. In the composite valve 120 of FIG. 5, the connection step occurs when the valve stem is insert molded into the metal head. The metal valve head can be formed on a screw machine or turned or spun on a lathe. If desired, the valve head can have a ceramic coating.

While the machining operations described above are preferably conducted after the injection molded engine part is post cured, one or more of these machining operations can be conducted before post curing if desired.

The composite engine part and the thermoplastic, amide-imide resinous polymer contained therein substantially maintain their shape, dimensional stability and structural integrity at engine operating conditions. Usual engine operating temperatures do not exceed 350° F. Oil cooled engine operating temperatures range from about 200° F. to 250° F. Advantageously, the composite thermoplastic, amide-imide resinous, polymeric engine part is impervious and chemically resistant to oil, gasoline, diesel fuel, and engine exhaust gases at engine operating conditions.

The thermoplastic resin in the composite engine part comprises 40% to 100%, preferably 65% to 75%, by weight amide-imide resinous polymer. The polymer is preferably reinforced with graphite fibers and/or glass fibers. In molded parts the fibers have an average length of 6 to 10 mils and a preferred diameter of about 0.2 to 0.4 mils. The ratio of the length to diameter of the fibers is from 2 to 70, averaging about 20. While the above fiber lengths and diameters are preferred for best structural strength, other lengths and diameters can be used, if desired. The graphite fibers can be granulated or chopped and can be optionally sized or coated with a polysulfone sizing or some other polymer which will maintain its structural integrity at engine operating conditions. The glass fibers can be milled or chopped and can be sized with silane or some other polymer that maintains its structural integrity at engine operating conditions. Chopped graphite and glass fibers are preferably sized, while granulated graphite fibers are preferably unsized.

Desirably, the thermoplastic, amide-imide resinous polymer comprises 10% to 50%, preferably 30% to

34%, by weight graphite fibers or 10% to 60%, preferably 30% to 34%, by weight glass fibers. The polymer can have as much as 3% and preferably  $\frac{1}{2}$ % to 1% by weight powdered or granular polytetrafluoroethylene (PTFE) and/or as much as 6% by weight titanium dioxide. In some circumstances it may be desirable to add more PTFE.

The polymer's molding characteristics and molecular weight can be controlled to facilitate polymerization with an additional monomer, such as trimellitic acid (TMA), and can be prepared with the desired flow properties by the methods described in Hanson U.S. Pat. No. 4,136,085, which is hereby incorporated by reference.

The polymer can be blended with graphite, glass, PTFE, and titanium dioxide by the method described in Chen U.S. Pat. No. 4,224,214, which is hereby incorporated by reference.

The most preferred amide-imide polymer is reinforced with 30% by weight graphite fibers and has the following engineering properties:

TABLE I

| Property                                       | Typical Value      | Units                                | ASTM Test Method |
|------------------------------------------------|--------------------|--------------------------------------|------------------|
| <u>Mechanical Properties</u>                   |                    |                                      |                  |
| <u>Tensile Strength</u>                        |                    | psi                                  | D1708            |
| @ -321° F.                                     | 22,800             |                                      |                  |
| @ 73° F.                                       | 29,400             |                                      |                  |
| @ 275° F.                                      | 22,800             |                                      |                  |
| @ 450° F.                                      | 15,700             |                                      |                  |
| <u>Tensile Elongation</u>                      |                    | %                                    | D1708            |
| @ -321° F.                                     | 3                  |                                      |                  |
| @ 73° F.                                       | 6                  |                                      |                  |
| @ 275° F.                                      | 14                 |                                      |                  |
| @ 450° F.                                      | 11                 |                                      |                  |
| <u>Tensile Modulus</u>                         |                    | psi                                  | D1708            |
| @ 73° F.                                       | 3,220,000          |                                      |                  |
| <u>Flexural Strength</u>                       |                    | psi                                  | D790             |
| @ -321° F.                                     | 45,000             |                                      |                  |
| @ 73° F.                                       | 50,700             |                                      |                  |
| @ 275° F.                                      | 37,600             |                                      |                  |
| @ 450° F.                                      | 25,200             |                                      |                  |
| <u>Flexural Modulus</u>                        |                    | psi                                  | D790             |
| @ -321° F.                                     | 3,570,000          |                                      |                  |
| @ 73° F.                                       | 2,880,000          |                                      |                  |
| @ 275° F.                                      | 2,720,000          |                                      |                  |
| @ 450° F.                                      | 2,280,000          |                                      |                  |
| <u>Compressive Strength</u>                    | 32,700             | psi                                  | D695             |
| <u>Shear Strength</u>                          |                    | psi                                  | D732             |
| @ 73° F.                                       | 17,300             |                                      |                  |
| <u>Izod Impact</u>                             |                    | ft.-lbs./in.                         | D256             |
| @ 73° F.                                       | 0.9                |                                      |                  |
| <u>Thermal Properties</u>                      |                    |                                      |                  |
| <u>Deflection Temperature</u>                  |                    | °F.                                  | D648             |
| @ 264 psi                                      | 540                |                                      |                  |
| <u>Coefficient of Linear Thermal Expansion</u> | $5 \times 10^{-6}$ | in./in./°F.                          | D696             |
| <u>Thermal Conductivity</u>                    | 3.6                | btu-in.<br>hr.-ft. <sup>2</sup> -°F. | C177             |
| <u>Flammability</u>                            | 94V0               | Underwriters Laboratories            | 94               |
| <u>Limiting Oxygen Index</u>                   | 52                 | %                                    | D2863            |
| <u>General Properties</u>                      |                    |                                      |                  |
| <u>Density</u>                                 | 1.42               | g/cc                                 | D792             |
| <u>Hardness "Rockwell" E</u>                   | 94                 |                                      |                  |
| <u>Water Absorption</u>                        | 0.26               | %                                    | D570             |

The preferred, glass reinforced, thermoplastic amide-imide resinous polymer comprises 30% by weight glass fibers and has the following properties:

TABLE II

| Property                                | Typical Value      | Units                                | ASTM Test Method |
|-----------------------------------------|--------------------|--------------------------------------|------------------|
| <u>Mechanical Properties</u>            |                    |                                      |                  |
| <u>Tensile Strength</u>                 |                    | psi                                  | D1708            |
| @ -321° F.                              | 29,500             |                                      |                  |
| @ 73° F.                                | 29,700             |                                      |                  |
| @ 275° F.                               | 23,100             |                                      |                  |
| @ 450° F.                               | 16,300             |                                      |                  |
| <u>Tensile Elongation</u>               |                    | %                                    | D1708            |
| @ -321° F.                              | 4                  |                                      |                  |
| @ 73° F.                                | 7                  |                                      |                  |
| @ 275° F.                               | 15                 |                                      |                  |
| @ 450° F.                               | 12                 |                                      |                  |
| <u>Tensile Modulus</u>                  |                    | psi                                  | D1708            |
| @ 73° F.                                | 1,560,000          |                                      |                  |
| <u>Flexural Strength</u>                |                    | psi                                  | D790             |
| @ -321° F.                              | 54,400             |                                      |                  |
| @ 73° F.                                | 48,300             |                                      |                  |
| @ 275° F.                               | 35,900             |                                      |                  |
| @ 450° F.                               | 26,200             |                                      |                  |
| <u>Flexural Modulus</u>                 |                    | psi                                  | D790             |
| @ -321° F.                              | 2,040,000          |                                      |                  |
| @ 73° F.                                | 1,700,000          |                                      |                  |
| @ 275° F.                               | 1,550,000          |                                      |                  |
| @ 450° F.                               | 1,430,000          |                                      |                  |
| Compressive Strength                    | 34,800             | psi                                  | D695             |
| <u>Shear Strength</u>                   |                    | psi                                  | D732             |
| @ 73° F.                                | 20,100             |                                      |                  |
| <u>Izod Impact</u>                      |                    | ft.-lbs./in.                         | D256             |
| @ 73° F.                                | 1.5                |                                      |                  |
| <u>Thermal Properties</u>               |                    |                                      |                  |
| <u>Deflection Temperature</u>           |                    | °F.                                  | D648             |
| @ 264 psi                               | 539                |                                      |                  |
| Coefficient of Linear Thermal Expansion | $9 \times 10^{-6}$ | in./in./°F.                          | D696             |
| Thermal Conductivity                    | 2.5                | btu-in.<br>hr.-ft. <sup>2</sup> -°F. | C177             |
| Flammability                            | 94V0               | Underwriters Laboratories            | 94               |
| Limiting Oxygen Index                   | 51                 | %                                    | D2863            |
| <u>Electrical Properties</u>            |                    |                                      |                  |
| <u>Dielectric Constant</u>              |                    |                                      | D150             |
| @ 10 <sup>3</sup> Hz                    | 4.4                |                                      |                  |
| @ 10 <sup>6</sup> Hz                    | 6.5                |                                      |                  |
| <u>Dissipation Factor</u>               |                    |                                      | D150             |
| @ 10 <sup>3</sup> Hz                    | .022               |                                      |                  |
| @ 10 <sup>6</sup> Hz                    | .023               |                                      |                  |
| Volume Resistivity                      | $6 \times 10^{16}$ | ohms-in.                             | D257             |
| Surface Resistivity                     | $1 \times 10^{18}$ | ohms                                 | D257             |
| Dielectric Strength                     | 835                | volts/mil.                           |                  |
| <u>General Properties</u>               |                    |                                      |                  |
| Density                                 | 1.56               | g/cc                                 | D792             |
| Hardness "Rockwell" E                   | 94                 |                                      |                  |
| Water Absorption                        | 0.24               | %                                    | D570             |

The amide-imide polymers are prepared by reacting an aromatic polycarboxylic acid compound (acyl halide carboxylic acid and/or carboxylic acid esters) having at least three carboxylic acid groups such as trimellitic acid (TMA), 4-trimellitoyl anhydride halide (4-TMAC), pyromellitic anhydride, pyromellitic acid, 3,4,3',4' benzophenone tetracarboxylic acid or an anhydride thereof, or oxybis benzene dicarboxylic acid or an anhydride thereof.

The amide-imide polymers are preferably prepared by reacting an acyl halide derivative of an aromatic tricarboxylic acid anhydride with a mixture of largely- or wholly-aromatic primary diamines. The resulting products are polyamides wherein the linking groups are predominantly amide groups, although some may be imide groups, and wherein the structure contains free

carboxylic acid groups which are capable of further reaction. Such polyamides are moderate molecular weight polymeric compounds having in their molecule units of:



and units of:



and, optionally, units of:



wherein the free carboxyl groups are ortho to one amide group, Z is an aromatic moiety containing 1 to 4 benzene rings or lower-alkyl-substituted benzene rings, R<sub>1</sub>, R<sub>2</sub> and R<sub>3</sub> are different and are divalent wholly- or largely-aromatic hydrocarbon radicals. These hydrocarbon radicals may be a divalent aromatic hydrocarbon radical of from 6 to about 10 carbon atoms, or two divalent aromatic hydrocarbon radicals each of from 6 to about 10 carbon atoms joined directly or by stable linkages such as -O-, methylene, -CO-, -SO<sub>2</sub>-, -S-; for example, -R'-O-R', -R'-CH<sub>2</sub>-R', -R'-CO-R', -R'-SO<sub>2</sub>-R' and -R'-S-R'.

The polyamides are capable of substantially complete imidization by heating by which they form the polyamide-imide structure having to a substantial extent reoccurring units of:



and units of:



and, optionally, units of:



wherein one carbonyl group is meta to and one carbonyl group is para to each amide group and wherein Z, R<sub>1</sub> R<sub>2</sub> and R<sub>3</sub> are defined as above. Typical copolymers of this invention have up to about 50 percent imidization prior to heat treatment, typically about 10 to about 40 percent.

The polyamide-imide copolymers are prepared from an anhydride-containing substance and a mixture of wholly- or partially-aromatic primary diamines. Usefully the anhydride-containing substance is an acyl halide derivative of the anhydride of an aromatic tricarboxylic acid which contains 1 to 4 benzene rings or lower-alkyl-substituted benzene rings and wherein two of the carboxyl groups are ortho to one another. More preferably, the anhydride-containing substance is an acyl halide derivative of an acid anhydride having a single benzene or lower-alkyl-substituted benzene ring, and most preferably, the substance is the acyl chloride derivative of trimellitic acid anhydride (4-TMAC).

Usefully the mixture of diamines contains two or more, preferably two or three, wholly- or largely-aromatic primary diamines. More particularly, they are wholly- or largely-aromatic primary diamines containing from 6 to about 10 carbon atoms or wholly- or largely-aromatic primary diamines composed of two divalent aromatic moieties of from 6 to about 10 carbon atoms, each moiety containing one primary amine group, and the moieties linked directly or through, for example, a bridging —O—, —S—, —SO<sub>2</sub>—, —CO—, or methylene group. When three diamines are used they are preferably selected from the class composed of:



said X being an —O—, —CH<sub>2</sub>—, or —SO<sub>2</sub>— group. More preferably, the mixture of aromatic primary diamines is two-component and is composed of meta-phenylenediamine (MPDA) and p,p'-oxybis(aniline) (OBA), p,p'-methylenebis (aniline) (MBA), and p,p'-oxybis(aniline), p,p'-sulfonylbis(aniline) (SOBA), and p,p'-oxybis(aniline), p,p'-sulfonylbis(aniline) and meta-phenylenediamine, or p,p'-sulfonylbis (aniline) and p,p'-methylenebis(aniline). Most preferably, the mixture of primary aromatic diamines contains meta-phenylenediamine and p,p'-oxybis(aniline). The aromatic nature of the diamines provides the excellent thermal properties of the copolymers while the primary amine groups permit the desired imide ring and amide linkages to be formed.

When two diamines are used to achieve a polymer usefully combining the properties of both diamines, it is usual to stay within the range of about 10 mole % of the first diamine and 90 mole % of the second diamine to about 90 mole % of the first diamine and 10 mole % of the second diamine. Preferably the range is about a 20 to 80 mole ratio to about an 80 to 20 mole ratio. In the preferred embodiment wherein the acyl chloride of

5 trimellitic acid anhydride is copolymerized with a mixture of p,p'-oxybis(aniline) and meta-phenylenediamine, the preferred range is from about 30 mole % of the former and about 70 mole % of the latter to about 70 mole % of the former and about 30 mole % of the latter.

10 Although embodiments of the invention have been shown and described, it is to be understood that various modifications and substitutions, as well as rearrangements of structural features and/or process steps, can be made by those skilled in the art without departing from the novel spirit and scope of this invention.

What is claimed is:

1. A composite engine valve, comprising:

a metal valve head for opening and closing an engine manifold communicating with a cylinder of an engine; and  
an elongated, thermoplastic, amide-imide resinous polymeric valve stem connected to said valve head said thermoplastic amide-imide valve stem and said metal valve head maintaining their structural integrity at engine operating conditions.

2. A composite engine valve in accordance with claim 1 wherein said valve head and said valve stem each define connection parts and one of said connection parts has a threaded stud extending outwardly therefrom and the other connection part has stud-receiving means for threadedly receiving said stud.

3. A composite engine valve in accordance with claim 2 wherein said stud-receiving means is an internally threaded hole.

4. A composite engine valve in accordance with claim 2 wherein said stud-receiving means includes a recess and a coil spring positioned within said recess for threadedly engaging said stud.

5. A composite engine valve in accordance with claim 4 wherein said valve head has said stud, and said valve stem has said coil spring and defines said recess.

6. A composite engine valve in accordance with claim 1 wherein said valve head defines a stem head-receiving cavity, and said valve stem has an enlarged insert molded stem head shaped generally complementary to and positioned within said cavity.

7. A composite engine valve in accordance with claim 1 wherein said valve head has a generally planar, circular disc, and said sidewalls have a general semi-hyperboloid shape.

8. A composite engine valve in accordance with claim 1 wherein said valve head and stem are substantially solid.

9. A composite engine valve in accordance with claim 1 wherein said metal is selected from the group consisting of aluminum and steel.

10. A composite engine valve in accordance with claim 1 wherein said amide-imide stem defines at least one keeper-receiving groove for receiving split keeper rings or locking keys which wedge against and connect a valve spring retainer to said amide-imide stem.

11. A composite engine valve in accordance with claim 1 wherein said metal comprises titanium.

12. A composite engine part in accordance with claim 1 wherein said valve stem comprises a reaction product of a trifunctional carboxylic acid compound and at least one diprimary aromatic diamine.

13. A composite engine part in accordance with claim 12 wherein said valve stem comprises at least one of the following moieties:



and



wherein one carbonyl group is meta to and one carbonyl group is para to each amide group and wherein Z is a trivalent benzene ring or lower-alkyl-substituted trivalent benzene ring, R<sub>1</sub> and R<sub>2</sub> are different and are divalent aromatic hydrocarbon radicals of from 6 to about 10 carbon atoms or two divalent aromatic hydrocarbon radicals of from 6 to about 10 carbon atoms joined directly or by stable linkages selected from the group consisting of —O—, methylene, —CO—, —SO<sub>2</sub>—, and —S— radicals and wherein said R<sub>1</sub> and R<sub>2</sub> containing units run from about 10 mole percent R<sub>1</sub> containing unit and about 90 mole percent R<sub>2</sub> containing unit to about 90 mole percent R<sub>1</sub> containing unit and about 10 mole percent R<sub>2</sub> containing unit.

14. A composite engine part in accordance with claim 13 wherein R<sub>1</sub> is



15. A composite engine part in accordance with claim 13 wherein Z is a trivalent benzene ring, R<sub>1</sub> is



R<sub>2</sub> is



and wherein the concentration range runs from about 30 mole percent of the R<sub>1</sub> containing units and about 70

mole percent of the R<sub>2</sub> containing units to about 70 mole percent of the R<sub>1</sub> containing units and about 30 mole percent of the R<sub>2</sub> containing units.

16. A composite engine part in accordance with claim 13 wherein said valve stem comprises from 40% to 100% by weight amide-imide resinous polymer.

17. A composite engine part in accordance with claim 16 wherein said valve stem comprises from 65% to 75% by weight amide-imide resinous polymer.

18. A composite engine part in accordance with claim 13 wherein said valve stem comprises a fibrous reinforcing material selected from the group consisting essentially of graphite and glass.

19. A composite engine part in accordance with claim 18 wherein said valve stem comprises from 10% to 50% by weight graphite.

20. A composite engine part in accordance with claim 19 wherein said valve stem comprises from 30% to 34% by weight graphite.

21. A composite engine part in accordance with claim 18 wherein said valve stem comprises 10% to 60% by weight glass.

22. A composite engine part in accordance with claim 21 wherein said valve stem comprises 30% to 34% by weight glass.

23. A composite engine part in accordance with claim 18 wherein said fibrous reinforcing material has a polymeric sizing that substantially maintains its structural integrity at engine operating conditions.

24. A composite engine part in accordance with claim 18 wherein said valve stem comprises not greater than 3% by weight polytetrafluoroethylene.

25. A composite engine part in accordance with claim 24 wherein said valve stem comprises from ½% to 1% by weight polytetrafluoroethylene.

26. A composite engine part in accordance with claim 18 wherein said valve stem comprises not more than 6% by weight titanium dioxide.

27. A process for forming a composite valve for use in an engine, comprising the steps of:

molding a thermoplastic, amide-imide resinous polymer to form an elongated valve stem;  
allowing said amide-imide valve stem to cool below its plastic deformation temperature;  
post curing said amide-imide valve stem by solid state polymerization to enhance the strength and integrity of said amide-imide valve stem;  
forming a metal valve head; and  
connecting said amide-imide valve stem to said metal valve head.

28. A process in accordance with claim 27 including cutting at least one keeper-receiving groove on said stem with a lathe.

29. A process in accordance with claim 27 wherein said valve head is formed at least in part on a screw machine.

30. A process in accordance with claim 29 including threading said valve head; drilling a recess in said stem;

60 and placing a coil spring in said recess; and wherein said connecting includes screwing the threaded portion of said valve head into said coil spring.

31. A process in accordance with claim 27 including grinding said head and said stem.

32. A process in accordance with claim 27 wherein said molding comprises injection molding.

33. A process in accordance with claim 27 wherein said valve head is formed with a cavity prior to said

molding; and said molding and said connecting are performed together by insert molding said valve stem into said cavity of said head.

34. A process in accordance with claim 27 wherein said valve head is formed on a lathe. 5

35. A process in accordance with claim 27 wherein said metal valve head is selected from the group consisting of aluminum, steel and titanium.

36. A process in accordance with claim 27 wherein said amide-imide polymer is prepared by reacting a trifunctional carboxylic acid compound with at least one diprimarily aromatic diamine. 10

37. A process in accordance with claim 36 wherein said amide-imide polymer comprises one of the following moieties: 15



and



wherein one carbonyl group is meta to and one carbonyl group is para to each amide group and wherein Z is a trivalent benzene ring or lower-alkyl-substituted trivalent benzene ring, R<sub>1</sub> and R<sub>2</sub> are different and are divalent aromatic hydrocarbon radicals of from 6 to about 10 carbon atoms or two divalent aromatic hydrocarbon radicals of from 6 to about 10 carbon atoms joined directly or by stable linkages selected from the group consisting of —O—, methylene, —CO—, —SO<sub>2</sub>—, and —S— radicals and wherein said R<sub>1</sub> and R<sub>2</sub> containing units run from about 10 mole percent R<sub>1</sub> containing unit and about 90 mole percent R<sub>2</sub> containing unit to about 90 mole percent R<sub>1</sub> containing unit and about 10 mole percent R<sub>2</sub> containing unit. 35

38. A process in accordance with claim 37 wherein R<sub>1</sub> is



-continued



39. A process in accordance with claim 37 wherein Z is a trivalent benzene ring, R<sub>1</sub> is



R<sub>2</sub> is



and wherein the concentration range runs from about 30 mole percent of the R<sub>1</sub> containing units and about 70 mole percent of the R<sub>2</sub> containing units to about 70 mole percent of the R<sub>1</sub> containing units and about 30 mole percent of the R<sub>2</sub> containing units.

40. A process in accordance with claim 37 wherein said polymer comprises from 10% to 50% by weight graphite fibers.

41. A process in accordance with claim 40 wherein said polymer comprises from 30% to 34% by weight graphite fibers.

42. A process in accordance with claim 37 wherein said polymer comprises from 10% to 60% by weight glass fibers.

43. A process in accordance with claim 42 wherein said polymer comprises from 30% to 34% by weight glass fibers.

44. A process in accordance with claim 36 wherein said polymer comprises a fibrous reinforcing material selected from the group consisting essentially of graphite and glass; and said fibrous reinforcing material is axially injected into a stem-shaped cavity of a mold and oriented in an axial direction in said cooled valve stem.

\* \* \* \* \*